

May 26, 1942.

C. A. LAISE

2,284,288

LAMP-MAKING METHOD

Original Filed June 7, 1939



FIG-2



*Inventor*

CLEMENS A. LAISE Deceased  
by FIDELITY UNION TRUST COMPANY executor

BY *Charles J. Holland*  
ATTORNEY

## UNITED STATES PATENT OFFICE

2,284,288

## LAMP-MAKING METHOD

Clemens A. Laise, deceased, late of Tenafly, N. J.,  
by Fidelity Union Trust Company, executor,  
Newark, N. J., assignor to Callite Tungsten  
Corporation, Union City, N. J., a corporation of  
Delaware

Original application June 7, 1939, Serial No.  
277,944. Divided and this application Decem-  
ber 3, 1940, Serial No. 368,308

4 Claims. (Cl. 176—13.2)

The present invention relates to a method of forming a tungsten filament of high efficiency adaptable for use in an electric incandescent lamp. An important feature of the invention resides in the fact that scavenging materials are included in the slug from which the filament is drawn, and the filament so formed is then given a heat treatment in an atmosphere of wet hydrogen whereby the scavenging materials are distilled out and all impurities are eliminated. The filament resulting from this treatment consists of long interlocking sections and can be operated at high efficiency and long life.

This application is a division of copending application Serial No. 277,944, filed June 7, 1939, by the executors of the last will and testament of Clemens A. Laise, deceased.

The expression "high efficiency" as used in the present application needs a certain definition. It is probably true that this term has been in use since the early days of the lamp art. It is certainly true that with the introduction of metallic filaments, the lamps utilizing these filaments became known as "high efficiency lamps." The term, however, had meaning only in comparison with carbon lamps and other lamps of lesser efficiency. With the appearance of the tungsten filament lamp, the term acquired a new meaning and when this was followed by the gas-filled lamp with a coiled tungsten filament, it was thought that a lamp of this type was the "high efficiency lamp."

Developments of recent years, however, have shown still higher efficiencies are possible. For, whereas in former times each increase in efficiency was attained by use of an improved filament material or by use of a more suitable gaseous atmosphere, it has lately been the aim to use the same gaseous atmosphere and the same filament material but to attain greater efficiency by applying more exact engineering principles to the lamp construction.

In the lamp art, efficiency consists in obtaining the greatest amount of lumens per watt consistent with a sufficiently long life to satisfy commercial and practical needs. As efficiency is increased the life of the lamp is shortened, other things being equal. In the lamp art of the past, however, the highest possible efficiency was rarely attained for the reason that such a lamp was not well adapted to sustain the shock of turning the current on or off. A metal filament is most conductive when cold; but as the temperature increases, the resistance also increases. There is, therefore, at the instant of switching on, a

sudden surge of current through the filament which produces a shock sufficient in many cases to rupture the filament.

It is an object of the present invention to provide as a product of said method a filament that, when used in a lamp, is capable of obtaining an extraordinarily high efficiency and a long commercial life. In Patent No. 1,631,493 issued to Clemens A. Laise on June 7, 1927, there is described and claimed a process of making a refractory metal product consisting of tungsten containing certain scavenging bodies such as boron nitride. When this metal was made into a slug it could be drawn down into a very fine grained filament suitable for an electric incandescent lamp. The finished filamentary body might contain as little as 1% and as high as 20% of boron nitride, and as such it formed a very suitable and efficient filament for an electric incandescent lamp of the time that patent was issued. The filament of the present invention may be considered as of the general type described and claimed in said Patent No. 1,631,493 in that the slug from which it is drawn consists mainly of tungsten but has an addition of boron nitride or boron suboxide and potassium borate, all of which have a scavenging effect. However, in contradistinction to said patent above mentioned, the metallic bar or slug from which the filament of this invention is drawn is so treated that at the sintering temperature a considerable portion of the scavenging materials distils out and takes along with it detrimental impurities that may be present in the tungsten base. The amount of such scavenger additions is such that in the final filament the amount remaining is very minute, being one-fourth of one per cent. or less.

The filament drawn from this slug so prepared is substantially pure tungsten, but owing to the treatment hereinbefore referred to and hereinafter more particularly described, the filament has few sectional boundaries, if any, in relation to its length. The filament metal is relatively soft and pliable and the sectional boundaries where they occur interlock laterally and longitudinally of the wire in such a manner that during burning in a lamp there is only very slight tendency to sag, offset or rupture, and, the intergranular cement being reduced to a minimum, the filament has little tendency to twist or distort after it has been shaped and set into suitably concentrated form. One prime cause of brittleness in tungsten filaments of the granular type of the prior art as represented in

Patent No. 1,631,493, and in most filaments of that time, is the presence of foreign non-metallic substances in the grain boundaries, and in the fact that the filaments have a very large number of small grains rather than large crystals such as are contemplated in the present invention. For instance, in the old pressed or squirted tungsten filaments, an organic binder was used which became carbonized during the process of manufacture and formed carbides in the crystal boundaries. In the drawn tungsten filaments as formerly produced, additions of various substances such as the oxides of calcium, aluminum or thorium were added for the purpose of retarding the growth of crystals. This practice resulted also in compounds in the grain boundaries that tended to produce a brittle filament, particularly after a short period of use. In the later, so-called non-sag tungsten filament, additions were made to the metal that produced silicon hydrides in the grain boundaries, with a resulting brittleness after relatively short use.

All such intergranular substances act solely as cements holding the grains together and preventing the grains from coalescing and forming larger grains. In the slug from which the filament of the present invention is drawn, however, the cementing material is composed of scavenging substances which were added to the tungsten powder from which the slugs are made. The slugs are worked into form in the usual way and the conditions of manufacture and heat treatment are so regulated that they have a grain count of approximately 15,000 to 20,000 grains per square millimeter.

The slugs are mechanically worked by swaging and drawing into wire, and then concentrated into coils or coiled coils or rolled into ribbon and corrugated or twisted into concentrated form. In making coiled coils of filament wire, the wire should be so wound that the magnetic effect due to the lines of force generated by it will not cause short-circuiting. When making coils or coiled coils, mandrels of nickel or nichrome or other refractory metals soluble in acids may be used, and the coil or coiled coil is heated on the mandrel in an atmosphere of wet hydrogen at temperatures ranging from 1000° C. to 1500° C. until a permanent set is imparted to the filament and the wire has been relieved of all of its strain. Thus, there will be no readjustment of the coil after the mandrel is dissolved out.

Wet hydrogen is used, a practice contrary to that of the present art in which dry hydrogen is used in such operations. Wet hydrogen tends to decompose any carbides that may be on the surface or in the grain boundaries of the filaments. If dry hydrogen is used, carbides are likely to form with the filament metal in the presence of carbon or carbon compounds. As a result of this process of using wet hydrogen, pliability and ductility of the filament is not impaired as it would be if dry hydrogen were used.

During the heat treatment above described, the scavenging materials tend to distil out, carrying with them substantially all impurities, including occluded hydrogen, that may be present in the grain boundaries. With these impurities eliminated there is little obstruction to rapid grain growth when the germinating temperature is reached, and accordingly the filament forms into long sections with but few interlocking section boundaries. Instead of the particular scavenging materials mentioned, other refractory

nitrides may be used with excellent effect, such as barium nitride and beryllium nitride.

The heat treated coil and mandrel are then cut to proper lengths to give the proper voltage of lamp and the mandrel is then dissolved in suitable acids such as nitric acid and sulphuric acid if nickel or nickel alloys are used as mandrel wire.

After the coil or other shape of filament treated in the above manner is mounted into the lamp, the lamp is sealed and exhausted or filled with gas and then flashed by connecting the lamp in series with a rheostat or nichrome resistance at about 125% over voltage, that is, 125% of the rated voltage of the filament for a period of about five minutes, so that the filament quickly attains the germinating temperatures and the grains coalesce or flow into each other, producing a light-emitting medium with long interlocking sections which have little tendency to sag or distort. Such sections may consist of at least one turn and preferably several turns of coil, especially after the lamp has burned about one hour at its rated voltage.

During the flashing operation it is desirable to use twice the voltage of the greatest voltage of the lamp and so regulate the proper voltage in this temporary circuit so that about 125% drop takes place across the lamp and 75% in the balance of the circuit consisting of a suitable rheostat.

In the drawing Fig. 1 illustrates a longitudinally sectional view of the filament of this invention, and Fig. 2 illustrates a cross-section thereof.

It is apparent that this filament of few interlocking sections can be operated at a much higher efficiency or lumen output and longer life than a highly crystallized filament of many grain boundaries. Furthermore, it retains its shape after it is once permanently set or flashed by my special process in the lamp circuit of this invention, so that it does not droop, shrink, twist or short-circuit between the individual sections.

The shape of my light-emitting filament may be a round cylindrical wire section, a square or oblong ribbon section, or may be in the form of ribbon corrugated or twisted or in the form of a coil or a double coil or helical coil. For gas-filled lamps, especially of the higher voltage type, a concentrated form such as a coiled-coil is desirable. In every case, however, my principle of treating the specially prepared filament body remains the same, namely, that the filament body containing boron scavengers, or the like, is subjected in my special circuit to a flashing or heat treating operation after the lamp is exhausted or even after it is based to produce the final structure in my light-emitting element as previously set forth.

The filament of this invention is preferably mounted upon lead wires of the general type described and claimed in the patent to Clemens A. Laise and Jacob Kurtz No. 2,120,561, dated June 14, 1938. Because of the exceptional heat and current conductivity characteristics of the material of these lead wires, they may be made much smaller in diameter than in the case of lead wires generally used in lamps of the present art of an equivalent wattage and may be as small as 50% of the cross-sectional area of the lead wire of such generally used lamps.

Having thus described the invention, what is claimed is:

1. The method of forming a concentrated tungsten filament which comprises drawing a filament from a tungsten slug containing scavenging material, then coiling the filament into coiled coils, then heating said coiled filament to 1000° C. to 1500° C. in an atmosphere of wet hydrogen, thereafter mounting said coiled filament in a lamp and flashing the same by connecting it in series with a resistance and impressing thereon a voltage of approximately 125% of the rated voltage of the lamp until the scavenging materials are substantially distilled out and the filament materials form into long interlocking grains.

2. The method of forming a concentrated tungsten filament by heating the same in an atmosphere of wet hydrogen, then mounting the filament in a lamp circuit having a resistance element in series with the filament, applying a difference of potential so as to instantaneously bring said filament to its germinating temperature and thereby causing the coalescence of the constituent grains into long interlocking sections.

3. The method of forming a filament of high efficiency comprising incorporating scavenging material in the filament-forming powder, forming the powder into a slug, drawing the slug into

5 a wire, coiling the wire, coiling the coils, heating said coils in an atmosphere of wet hydrogen, and then mounting the filament in a lamp circuit having a resistance element in series with the filament and applying thereto a difference of potential so as to instantaneously bring said filament to its germinating temperature, thereby first causing the distillation and elimination of impurities from the grain boundaries and then causing the coalescence of its constituent grains into relatively long interlocking sections.

10 20 4. The method of forming a concentrated filament which comprises drawing a filament from a tungsten slug containing scavenging materials, concentrating the filament, heat treating the concentrated filament at a temperature of 1000° C. to 1500° C. in an atmosphere of wet hydrogen, and then heating said filament by connecting it in series with a resistance to the germinating temperature in a suitable atmosphere until said scavenging materials are substantially distilled out and the filament forms large interlocking grains.

FIDELITY UNION TRUST COMPANY,  
By LESLIE G. McDOUALL,  
Vice-President  
Sole Surviving Executor of the Last Will and  
Testament of Clemens A. Laise, Deceased.